

# UNITED STATES PATENT OFFICE.

SIGMOND SAXE, OF NEW YORK, N. Y.

## SILK-DYEING.

1,263,126.

Specification of Letters Patent. Patented Apr. 16, 1918.

No Drawing.

Application filed August 16, 1917. Serial No. 186,543.

To all whom it may concern:

Be it known that I, SIGMOND SAXE, a citizen of the United States, residing at New York, in the county of New York and State 5 of New York, have invented certain new and useful Improvements in Silk-Dyeing, of which the following is a specification.

This invention relates to silk dyeing; and it comprises a method of weighting silk and 10 toning the colors of dyed silk, and particularly to "jetting" black silks, where silk is preliminarily dyed and is then worked in a strong decoction of the wood of Osage orange (*Maclura aurantiaca*) to which may be 15 added a small amount of tin crystals, the silk being thereafter mordanted and dyed; all as more fully hereinafter set forth and as claimed.

In the dyeing and weighting of silk many 20 substances have been proposed and used; and to some extent these additions have also been employed for the purpose of correcting the tone or hue of the dye; this being particularly the case in securing jet blacks. One 25 of the materials which is extensively used for the combined purpose of weighting and toning is what is known as gambier or catch. Gambier adds somewhat to the weight of the silk and in the case of black-dyed silks. 30 it brings the tone of the black nearer the jet black desired. It is therefore sometimes called a "jetting" agent. Gambier used alone gives the silk a brown color and in combination with dyes giving a blue black, 35 the result is nearly, but not exactly, a jet black. It gives only approximately the result desired. Gambier is however an undesirable material for dyeing purposes in many other respects, being a very crude material 40 containing much dirt and of an irregular quality. Ordinary or common gambier, which is the grade used by the silk trade, is usually sold without guarantee and without analysis.

45 I have found that if I replace the gambier in the ordinary silk dyeing operations with an extract of Osage orange (*Maclura aurantiaca*); I secure much more uniform and definite results and in addition I secure 50 better dyeing and weighting effects. An Osage orange extract may be substituted for gambier with good results in producing other dyes than blacks; but its advantages are most apparent in making jet blacks.

55 The Osage orange is a shrub or small tree, indigenous to this country and cultivated to

some extent for hedge purposes. It has practically no other utility. I have found that by extracting the wood with water, I can make an extract rich in tannin and dyeing a yellow color. I may make this extract in a diffusion apparatus or in other well known ways. Ordinarily I thereafter concentrate the extract to a relatively high density *in vacuo* or in other ways. Usually, 60 I concentrate it to the density of about 51° Twaddell to make a commercial preparation.

I use this Osage orange extract in dyeing silk. In and of itself it gives the silk a 70 yellow color and adds to the weight of the silk. Ordinarily, however, I do not use it alone as a dyestuff, but employ it in conjunction with other materials.

In one specific embodiment of my invention in weighting and in black-dyeing silk I first work the silk in a bath of nitrate of iron and treat with ferrocyanid or the like to produce a blue (Prussian blue). After this, I work the silk in a strong extract of 75 Osage orange, say, the extract of about the 51° Twaddell strength before mentioned. To this extract I may, or may not, add a small amount of tin crystals. The silk absorbs a large amount of solid matter from 80 the solution and is weighted about 50 per cent. After this, I add pyrolignite of iron or nitrate of iron and dye in the usual manner to produce a black. Because of the tone 85 imparted by the matters contained in the Osage orange extract, this final black will be a jet black and because of the superior weighting properties of Osage orange the silk will be of a better merchantable weight.

I find that about two-thirds of a pound of 90 Osage orange extract of 51° Twaddell will produce about the same weighting and dyeing effect as a pound of gambier as gambier runs. As stated gambier is a very irregular material, but in a general way the above relation may be said to exist. The black produced however is much better than that obtained with gambier. The results also are much more uniform, it being possible to reproduce exactly the same shades; while this 95 is not possible where different lots of ordinary gambier are employed.

The 51° Osage orange extract referred to gives an analysis showing about 45 per cent. water to 55 per cent. total solids; practically all of this solid matter being in solution. Of this amount some 39 per cent. responds to

the tests for tannin and about 12 per cent. is what may be called soluble non-tannins.

What I claim is:—

1. The process of dyeing and weighting silk which comprises treating such silk with a strong extract of wood of Osage orange.
- 5 2. The process of dyeing and weighting

silk a jet black which comprises mordanting and dyeing such silk, working in a strong extract of Osage orange and there-<sup>10</sup> after completing the black-dyeing.

In testimony whereof, I affix my signature.

SIGMOND SAXE.